

Patented Nov. 4, 1952

2,616,837

# UNITED STATES PATENT OFFICE

2,616,837

## PROCESS OF AIR-BLOWING ASPHALT

Joseph Carl Roediger, Brooklyn, N. Y., assignor to Standard Oil Development Company, a corporation of Delaware

No Drawing. Application January 3, 1949,  
Serial No. 69,031

3 Claims. (Cl. 196—74)

**1** The object of this invention is a process of air blowing asphalt to modify it to one having unexpected and desirable high flash points.

It is well known in the art to use asphaltic compositions as binders for mineral aggregates in the preparation of paving mixtures and as saturants and coatings in the preparation of roll and shingle roofings and in built-up roofings. Asphalt found naturally or prepared from petroleum crude oil both by direct distillation of an asphaltic crude oil or from a cracked petroleum oil may be used.

The manufacture of prepared roofing, the saturation of fibrous board, the preparation of certain types of asphalt paving mixtures, etc., require the heating of the asphalt to a fluid condition and therefore it is very desirable that the flash point of the asphalt being used be relatively high, preferably above 500° F., so that the manufacturing operation can be conducted with safety and freedom from flash fires.

Heretofore the production of asphalts having a satisfactory high flash point and other desirable properties has been a serious problem. The flash point of the asphalts produced by direct distillation to a large degree is dependent upon the type of compounds which exist in the crude oil as delivered from the well. For this reason, the asphalts obtainable from certain crude oils are too low in flash point to make them suitable for all general applications. One procedure followed in preparing asphalts of desirable characteristics from crude petroleum oil which produces a low flash asphalt is to reduce this by conventional means to a high flash point, high softening point asphalt bottoms. In other words, remove the major portion of the low boiling oils. These high softening point asphalt bottoms may then be blended with a high flash oil obtained in the processing of a crude oil of different origin. In this manner the final blended asphalt will have a higher flash point than that which is directly obtainable from the original asphaltic crude.

While this procedure will produce asphalts of satisfactory characteristics and having satisfactory flash points, certain problems are encountered. One difficulty is that it is generally uneconomical since double processing is required and two crudes must be handled.

According to this invention it was found that when selected silicones are added to the asphaltic composition the flash point of the asphalt is materially raised. The silicones used have a formula:



wherein R may be an alkyl or aryl group, m may be an integer of 1, 2 or 3, y is a variable integer whose value depends on m, the valency of Si be-

ing 4, and x is an integer greater than 2. Silicones having a viscosity at 77° F. of 100 to 1000 centistokes and flash of 600°-640° F. are used. For example, it is preferred to use a silicone oil having a viscosity of about 350 centistokes at 77° F. preferably from .0005 to .005% of the silicone oil based on the asphalt.

My invention may be readily understood by the following examples illustrating embodiments of the same.

### Example 1

Various percentages of a silicone oil polymer were used with Colombian and Venezuelan asphalts of the 80/100 penetration 77° F./100g./5 seconds grade commonly used for highway pavement construction. The results secured are as follows:

| 20                                   | Asphalt Crude Base                  | Asphalt Compositions |            |       |       |
|--------------------------------------|-------------------------------------|----------------------|------------|-------|-------|
|                                      |                                     | Colombian            | Venezuelan |       |       |
| 25                                   | Percent Methyl Polysiloxane Polymer | 0                    | 0.001      | 0     | 0.001 |
| Spec. Grav., 60° F.                  | 1.009                               | 1.007                | 1.025      | 1.023 |       |
| Flash (COC), °F.                     | 605                                 | 670                  | 595        | 700+  |       |
| Softening Point, °F.                 | 118                                 | 116                  | 117        | 117   |       |
| Penetration, 77° F./100 g./5 seconds | 84                                  | 83                   | 81         | 85    |       |
| Penetration, 32° F./100 g./5 seconds | 18                                  | 17                   | 19         | 19    |       |

From the above it is apparent that the flash points of the respective asphalts were increased to an appreciable degree without significant change in the other properties, aside from a slight reduction in specific gravity.

### Example 2

In other experiments various percentages of this polymer were added to Colombian and Venezuelan asphalts of the type used by the roofing industry for the saturation of the felt sheet forming the base for roll roofings. The results of these experiments are tabulated below:

| 45                                   |     | Asphalt Base |       |       |            |        |  |
|--------------------------------------|-----|--------------|-------|-------|------------|--------|--|
|                                      |     | Colombian    |       |       | Venezuelan |        |  |
| Percent Silicone Oil Polymer         | 0   | 0.0005       | 0.001 | 0.005 | 0          | 0.0005 |  |
| Flash (COC), °F.                     | 560 | 610          | 610   | 500   | 555        | 660    |  |
| Softening Point, °F.                 | 104 | 102          | 103   | 104   | 118        | 117    |  |
| Penetration, 77° F./100 g./5 seconds | 184 | 187          | 187   | 189   | 102        | 103    |  |
| Penetration, 32° F./100 g./5 seconds | 50  | 58           | 53    | 55    | 43         | 29     |  |

In the case of the Colombian asphalt polymer mixtures, maximum flash point increase is obtained within the range of 0.0005 to 0.001% added siloxane polymer. In other words, the optimum

increase in flash point occurs within a rather restricted range of polymer concentration.

Asphalt-silicone oil mixtures of this type can be used for the more efficient saturation of roofing felt, Celotex-type board and other fibrous boards since the higher flash point of this mixture permits operation with safety at higher saturating temperatures. Likewise, the higher operating temperature now possible permits the use of saturants of higher consistency than heretofore.

*Example 3*

Additional tests were run using a grade of asphalt flux which is subsequently air blown (oxidized) for the production of a roofer's flux, or by longer air blowing for the production of coating asphalt. The Lagunillas crude source flux having a 465° flash point used in these tests, produces by air blowing a roofer's flux and a coating asphalt which do not meet the usual specifications requiring a flash point in excess of 500° F., as shown in column A of the following tabulation.

|                                             | Lagunillas Flux (465° F. Flash) |       |
|---------------------------------------------|---------------------------------|-------|
| Percent Silicone Oil Polymer.....           | 0.0                             | 0.001 |
| I. Flux Base.....                           | A                               | B     |
| Flash (COC), °F.....                        | 465                             | 505   |
| Fire (COC), °F.....                         | 525                             | 585   |
| Furol Viscosity at 210° F.....              | 165                             | 161   |
| II. Roofer's Flux Oxidized from (I).....    | A                               | B     |
| Flash (COC), °F.....                        | 475                             | 520   |
| Fire (COC), °F.....                         | 525                             | 575   |
| Softening Point, °F.....                    | 109                             | 107   |
| Penetration, 77° F./100 g./5 seconds.....   | 172                             | 182   |
| Penetration, 32° F./100 g./5 seconds.....   | 73                              | 65    |
| III. Coating Asphalt Oxidized from (I)..... | A                               | B     |
| Flash (COC), °F.....                        | 500                             | 580   |
| Fire (COC), °F.....                         | 560                             | 605   |
| Softening Point, °F.....                    | 221                             | 226   |
| Penetration, 77° F./100 g./5 seconds.....   | 18                              | 13    |
|                                             | 13                              | 13    |

In the above table the roofer's flux compositions, item II, were made by conventional oxidation from the flux base, I. Similarly, the coating asphalt compositions, item III, were also made

by oxidation to a higher softening point asphalt from flux base, item I. In both the A and B series, the oxidations were carried out under identical conditions employing a 450° F. ±10° F. for the oxidation to Roofer's Flux and a 450/475° F. temperature when air blowing the Roofer's Flux to high SP Coating asphalt. These compositions were prepared using flux base without polymer addition for the A series and with 0.001% silicone polymer for the B series.

The above example also shows that the effectiveness of the silicone oil addition is not decreased when the flux-polymer composition is subjected to oxidation at elevated temperatures for the production of higher softening point oxidized asphalts.

What is claimed:

1. In the process of air-blowing asphalt, the improvement which comprises conducting said air-blowing in the presence of an amount of a methylpolysiloxane sufficient to substantially increase the flash point of said asphalt.

2. In the process of air-blowing asphalt, the improvement which comprises conducting said air-blowing in the presence of about 0.0005% to 0.005% of a methylpolysiloxane to substantially increase the flash point of said asphalt.

3. In the process of air-blowing asphalt, the improvement which comprises heating said asphalt to a temperature of about 450° F. and conducting said air-blowing in the presence of an amount of a methylpolysiloxane sufficient to substantially increase the flash point of said asphalt.

JOSEPH CARL ROEDIGER.

**REFERENCES CITED**

The following references are of record in the file of this patent:

**UNITED STATES PATENTS**

| Number    | Name            | Date          |
|-----------|-----------------|---------------|
| 2,258,218 | Rochow          | Oct. 7, 1941  |
| 2,416,504 | Trautman et al. | Feb. 25, 1947 |

**OTHER REFERENCES**

45. Oil and Gas Journal, October 6, 1945, pages 87 and 88.

Dow Corning Silicone Note Book Fluid Series No. 3, September 1948, page 11.